# EUROPEAN PATENT SPECIFICATION

(11) **EP 0 591 361 B1**
(45) Date of publication and mention of the grant of the patent: **27.12.1996**
(21) Application number: 92913760.2
(22) Date of filing: 02.06.1992
(51) Int. Cl.: D06P 1/40, D06P 3/06, D06P 3/24, D06P 1/00

(54) **METHOD FOR DYEING NYLON FILAMENTS**
Verfahren zur Färbung von Nylonspinnfäden
PROCEDE PERMETTANT DE TEINDRE DES FILAMENTS DE NYLON

(30) Priority: 17.06.1991 US 716196
(43) Date of publication of application: 13.04.1994
(73) Proprietor: GILLETTE CANADA INC., Kirkland, Quebec (CA)
(72) Inventor: SUHONEN, Christopher, H., San Jose, CA 95125 (US)
(74) Representative: Baillie, Iain Cameron
(86) International application number: US9204589
(87) International publication number: WO9222699

(56) References cited:
- US-A- 2 558 992
- US-A- 4 802 255
- US-A- 5 061 290
- CHEMICAL ABSTRACTS, vol. 104, no. 18, 5 May 1986, Columbus, Ohio, US; abstract no. 150660v, BARYBINA, L. A. ET AL 'Multiple use of residual dye solutions'

## Description

The invention relates to filaments for toothbrushes.

Breuer et al., U.S. Pat. No. 4,802,255 describes nylon monofilaments that include at least two colored regions, one of which is provided by a dye. The monofilaments are included in the bristles of toothbrushes and, as the toothbrush is used by the owner, the color intensity of the dyed region changes in response to wear, providing an indication of when the toothbrush should be replaced. Breuer et al. lists six food dyes or colorants that can be used to dye the monofilaments including Indigotine (FD&C Blue No. 2), and in col. 4 broadly describes the conditions that can be used for dyeing. Breuer et al. also provides a number of specific examples of dyeing procedures, including three (examples 4-6) in which Indigotine is used as the dye.

The specific dyeing procedures described by Breuer et al. were for laboratory samples. However, to produce a sufficient amount of dyed filaments for commercial toothbrushes, a procedure is needed that can be used for dyeing large amounts of filaments. The procedure should be cost-efficient and, of course, should produce nylon filaments that have a consistent level of dye penetration.

In general, the invention is a method for dyeing batches of nylon filaments for toothbrushes. As used herein, a batch is at least 0.9 kg (two pounds) of nylon filament. The method includes immersing a batch of a first nylon filament for between 10 minutes and 80 minutes in an aqueous solution containing between .01% and 0.1% weight to volume of Indigotine dye. The solution should have a pH between 1 and 7, and should have a temperature between 50°C. and 90°C. While the nylon filament is immersed, the dye penetrates into an outer cross-sectional region but not into an inner cross-sectional region. The batch of the first nylon filament is removed from the solution, and can be used for bristles in a wear-indicating toothbrush. The same procedure is repeated for a batch of a second nylon filament, reusing the same solution. Preferably, the same solution is then used for dyeing additional batches. In the preferred method, the aqueous solution contains between 0.01% and 0.05% weight to volume of Indigotine dye; the solution has a pH of between 2.5 and 4.5; and the temperature of the solution is between 70°C. and 85°C. Preferably, the dyeing step is performed at atmospheric pressure and takes less than 60 minutes, and the nylon filaments have a diameter of between 0.13 mm (0.005 inches) and 0.36 mm (0.014 inches).

The method can be used to produce commercial quantities of nylon filaments for use in wear-indicating toothbrushes in a cost-effective manner. For example, the procedure can be used on 4.5-18 kg (10-40 lb.) bathes of nylon filaments, and even on batches weighing 45 kg (100 lbs) or more. Importantly, the same solution can be reused at least once, and even up to five or six times, and still produce filaments in which the Indigotine dye has penetrated an even, consistent cross-sectional area. The method is easy to carry out, safe, and provides a stable dye solution.

Other advantages of the invention will be apparent from the description of the preferred embodiment thereof, and from the claims.

Dyed wear-indicating nylon monofilaments, toothbrushes including such monofilaments, and the way the toothbrushes are made are described in detail in Breuer et al.

The dyeing solution used in the method of the invention contains between 0.01% and 0.1% weight to volume Indigotine. If too much Indigotine is used, too much dye penetrates too far into the filament. If too little dye is used, too little dye may penetrate, and the solution may not be reusable because the initial batch of filament may absorb the limited quantity of dye present.

The temperature of the solution should be between 50°C. and 90°C. Too high a temperature results in water quickly evaporating off, resulting in the dye becoming more concentrated, and the dye being taken up too fast, making the degree of penetration more difficult to control. Too low a temperature results in too slow a dye uptake.

The dyeing process preferably is done at atmospheric pressure, to avoid the necessity of using large pressurized equipment in a plant.

Indigotine is an acid stable dye, and the solution should be acidic.

The volume of dyeing solution should be large enough so that the first batch of filament does not absorb such a high percentage of the dye in the solution that the solution cannot be reused to dye a second batch.

The nylon filaments, most preferably monofilaments, should be of the diameter commonly used in toothbrushes, most preferably 0.20 mm (0.008) or 0.23 mm (0.009 inch).

The nylon filament should be immersed in solution long enough to get adequate dye penetration of the outer cross-sectional diameter of the filament to provide good wear-indicating characteristics. Preferably, the immersion time should be as limited as possible, and should be less than 1 hour.

A detailed description of the most preferred method is provided below, beginning with a description of the equipment and solutions used, followed by the procedure.

The dyeing step is performed in a 2396 l (633 gallon) Whiting stainless steel tank having side dimensions of 762 x 1016 x 3302 mm (30" x 40" x 130").

The dyeing solution used in the tank includes 2 396 l (633 gallons) of distilled water; 7.7 liters of glacial acidic acid; and 555 g of 100% pure Indigotine. The temperature of the solution is maintained at 75°C. ± 1.5°C.

Two 2396 l (633 gallon) rinse tanks also are used. The first tank is filled with tap water. The second tank is filled with tap water mixed with 1.5 liters of Dow Corning #24 silicone emulsion.

The monofilament used is a 2.5 m (an eight foot) long, 0.20 mm (0.008 inch) diameter Wytex 6.12 S nylon hank (bundle) weighing approximately 4.5 kg (10 pounds). The hank should be siliconed, annealed, wet, and combed prior to dyeing, according to standard procedures. The hank should not be dried prior to use.

### Dyeing Procedure

1) Completely submerse four hanks in the dye solution.
2) Set timer for 45 minutes.
3) Lift and resubmerse hanks every 1.5 minutes to permit circulation of dye between filaments.
4) After 45 minutes, remove hanks and transfer to the first rinse tank. Rinse by dipping 4 to 5 times.
5) Transfer the to the second rinse tank. Continue rinsing by dipping another 4 to 5 times. This rinse will restore the finish lost during the dyeing process.
6) Recomb hanks and continue with the normal drying and wrapping process.
7) Repeat the procedure 4 times for additional batches of hanks, using the same solutions. The dye solution and first rinse are changed after 5 hanks have been dyed; the second rinse solution is replaced daily.
Optionally, the above procedure can be modified by immersing set of hanks for 30 minutes in a dyeing solution heated to 80°C. ± 1.5°C. In addition, the procedure can be used to dye 10 hanks at a time, as opposed to four hanks.

Other embodiments are within the claims.

## Claims

1. A method of dyeing nylon filaments for toothbrushes, comprising :
(a) wetting said nylon filaments and immersing a first batch of said nylon filament for between 10 minutes and 80 minutes in an aqueous solution comprising between 0.01% and 0.19% weight to volume of Indigotine dye, said solution having a pH between 1 and 7 and having a temperature between 50°C. and 90°C., said Indigotine dye consistently penetrating into said nylon filament to color an even outer cross-sectional region of said nylon filament, and not penetrating into an inner cross-sectional region of said nylon filament;
(b) removing the first batch of said nylon filament from said solution to provide a nylon filament having said outer cross-sectional region colored with said Indigotine dye and said inner cross-sectional region not colored with said Indigotine dye;
(c) repeating steps (a) and (b) for a second batch of said nylon filament, reusing the same said solution, said Indigotine dye consistently penetrating into said nylon filament to color evenly the same outer cross-sectional region of said nylon filament in said second batch as was colored in said first batch.

2. The method of claim 1, comprising the additional step of repeating steps (a) and (b) for a third batch of said nylon filament, reusing the same said solution, said Indigotine dye consistently penetrating into said nylon filament to color evenly the same outer cross-sectional region of said nylon filament in said third batch as was colored in said first batch.

3. The method of claim 2, comprising the additional step of repeating steps (a) and (b) for a fourth batch of said nylon filament, reusing the same said solution, said Indigotine dye consistently penetrating into said nylon filament to color evenly the same outer cross-sectional region of said nylon filament in said fourth batch as was colored in said first batch.

4. The method of claim 1, wherein step (a) is performed at atmospheric pressure.

5. The method of claim 1, wherein said solution has a temperature of between 70°C. and 85°C.

6. The method of claim 1, wherein said solution comprises between 0.01% and 0.05% weight to volume of Indigotine dye.

7. The method of claim 1, wherein said solution has a pH of between 2.5 and 4.5.

8. The method of claim 1, wherein said nylon filaments have an average diameter of between 0.127 and 0.356 mm (0.005 inches and 0.014 inches).

9. The method of claim 1, comprising the additional steps of affixing the first dyed nylon filament to the head of a toothbrush, and at least some of the second dyed nylon filament to the head of a toothbrush.

10. The method of claim 1, wherein said nylon filaments are monofilaments.

11. The method of claim 1, wherein said first batch of said nylon filament is immersed in said aqueous solution for less than 60 minutes.

12. The method of claim 1, wherein said first batch of said nylon filament weighs at least 4.8 kg (10 lbs.).

## Patentansprüche

1. Verfahren zum Färben von Nylonspinnfäden für Zahnbürsten, wobei das Verfahren die folgenden Schritte umfaßt:
(a) Anfeuchten der genannten Nylonpinnfäden und Eintauchen einer ersten Beschickung des genannten Nylonspinnfadens über einen Zeitraum von 10 Minuten bis 80 Minuten in eine wäßrige Lösung, die 0,01 bis 0,19 Volumengewichtsprozent des Farbstoffs Indigoblau umfaßt, wobei die genannte Lösung einen pH-Wert zwischen 1 und 7 sowie eine Temperatur zwischen 50°C und 90°C aufweist, wobei der genannte Farbstoff Indigoblau gleichmäßig in den genannten Nylonspinnfaden eindringt, um einen gleichmäßigen äußeren Querschnittsbereich des genannten Nylonspinnfadens zu färben, und wobei der Farbstoff nicht in einen inneren Querschnittsbereich des genannten Nylonspinnfadens eindringt;
(b) Entfernen der ersten Beschickung des genannten Nylonspinnfadens aus der genannten Lösung, so daß ein Nylonspinnfaden vorgesehen wird, der den genannten, mit dem genannten Farbstoff Indigoblau gefärbten äußeren Querschnittsbereich und den genannten, nicht mit dem Farbstoff Indigoblau gefärbten inneren Querschnittsbereich aufweist;
(c) Wiederholen der Schritte (a) und (b) für eine zweite Beschickung des genannten Nylonspinnfadens, wobei dafür die gleiche Lösung verwendet wird, wobei der genannte Farbstoff Indigoblau gleichmäßig in den genannten Nylonspinnfaden eindringt, um in der zweiten Beschickung den gleichen äußeren Querschnittsbereich des genannten Nylonspinnfadens gleichmäßig zu färben, wie bei der ersten Beschickung.

2. Verfahren nach Anspruch 1, wobei das Verfahren den zusätzlichen Schritt der Wiederholung der Schritte (a) und (b) für eine dritte Beschickung des genannten Nylonspinnfadens umfaßt, wobei dafür die gleiche Lösung verwendet wird, wobei der genannte Farbstoff Indigoblau gleichmäßig in den genannten Nylonspinnfaden eindringt, um in der dritten Beschickung den gleichen äußeren Querschnittsbereich des genannten Nylonspinnfadens gleichmäßig zu färben, wie bei der ersten Beschickung.

3. Verfahren nach Anspruch 2, wobei das Verfahren den zusätzlichen Schritt der Wiederholung der Schritte (a) und (b) für eine vierte Beschickung des genannten Nylonspinnfadens umfaßt, wobei dafür die gleiche Lösung verwendet wird, wobei der genannte Farbstoff Indigoblau gleichmäßig in den genannten Nylonspinnfaden eindringt, um in der vierten Beschickung den gleichen äußeren Querschnittsbereich des genannten Nylonspinnfadens gleichmäßig zu färben, wie bei der ersten Beschickung.

4. Verfahren nach Anspruch 1, wobei der Schritt (a) bei Atmosphärendruck durchgeführt wird.

5. Verfahren nach Anspruch 1, wobei die genannte Lösung eine Temperatur zwischen 70°C und 85°C aufweist.

6. Verfahren nach Anspruch 1, wobei die genannte Lösung zwischen 0,01 bis 0,05 Volumengewichtsprozent des Farbstoffs Indigoblau aufweist.

7. Verfahren nach Anspruch 1, wobei die genannte Lösung einen pH-Wert zwischen 2,5 und 4,5 aufweist.

8. Verfahren nach Anspruch 1, wobei die genannten Nylonspinnfäden einen durchschnittlichen Durchmesser zwischen 0,127 und 0,356 mm (0,005 Inch bis 0,014 Inch) aufweisen.

9. Verfahren nach Anspruch 1, wobei das Verfahren den zusätzlichen Schritt der Befestigung des ersten gefärbten Nylonspinnfadens an dem Kopf einer Zahnbürste und wenigstens eines Teils des genannten zweiten gefärten Nylonspinnfadens an dem Kopf einer Zahnbürste umfaßt.

10. Verfahren nach Anspruch 1, wobei es sich bei den genannten Nylonspinnfäden um Einzelfäden handelt.

11. Verfahren nach Anspruch 1, wobei die genannte erste Beschickung des genannten Nylonspinnfadens über einen kürzeren Zeitraum als 60 Minuten in die genannte wäßrige Lösung eingetaucht wird.

12. Verfahren nach Anspruch 1, wobei die genannte erste Beschickung des genannten Nylonspinnfadens mindestens 4,8 kg (10 Pfund) wiegt.

## Revendications

1. Procédé de teinture de filaments de Nylon pour brosses à dents, comprenant :
(a) le mouillage desdits filaments de Nylon et l'immersion d'un premier lot dudit filament de Nylon pendant 10 min à 80 min dans une solution aqueuse comprenant 0,01 % à 0,19 % en masse par volume de colorant indigotine, ladite solution ayant un pH compris entre 1 et 7 et ayant une température comprise entre 50°C et 90°C, ledit colorant indigotine pénétrant uniformément dans ledit filament de Nylon pour colorer une région en section droite externe uniforme dudit filament de Nylon, et ne pénétrant pas dans une région en section droite interne dudit filament de Nylon ;
(b) le retrait dudit premier lot dudit filament de Nylon de ladite solution pour fournir un filament de Nylon ayant ladite région en section droite externe colorée avec ledit colorant indigotine et ladite région en section droite interne non colorée avec ledit colorant indigotine ;
(c) la répétition des étapes (a) et (b) pour un second lot dudit filament de Nylon, en réutilisant la même solution, ledit colorant indigotine pénétrant uniformément dans ledit filament de Nylon pour colorer uniformément dans ledit second lot la même région en section droite externe dudit filament de Nylon que celle qui a été colorée dans ledit premier lot.

2. Procédé selon la revendication 1, comprenant l'étape supplémentaire de répétition des étapes (a) et (b) pour un troisième lot dudit filament de Nylon, en réutilisant la même solution, ledit colorant indigotine pénétrant uniformément dans ledit filament de Nylon pour colorer uniformément dans ledit troisième lot la même région en section droite externe dudit filament de Nylon que celle qui a été colorée dans ledit premier lot.

3. Procédé selon la revendication 2, comprenant l'étape supplémentaire de répétition des étapes (a) et (b) pour un quatrième lot dudit filament de Nylon, en réutilisant la même solution, ledit colorant indigotine pénétrant uniformément dans ledit filament de Nylon pour colorer uniformément dans ledit quatrième lot la même région en section droite externe dudit filament de Nylon que celle qui a été colorée dans ledit premier lot.

4. Procédé selon la revendication 1, dans lequel l'étape (a) est réalisée à la pression atmosphérique.

5. Procédé selon la revendication 1, dans lequel ladite solution a une température comprise entre 70°C et 85°C.

6. Procédé selon la revendication 1, dans lequel ladite solution comprend 0,01 % à 0,05 % en masse par volume de colorant indigotine.

7. Procédé selon la revendication 1, dans lequel ladite solution a un pH compris entre 2,5 et 4,5.

8. Procédé selon la revendication 1, dans lequel lesdits filaments de Nylon ont un diamètre moyen compris entre 0,127 et 0,356 mm (0,005 pouce et 0,014 pouce).

9. Procédé selon la revendication 1 comprenant les étapes supplémentaires de fixation du premier filament de Nylon teint à la tête d'une brosse à dents et au moins une certaine quantité du second filament de Nylon teint à la tête d'une brosse à dents.

10. Procédé selon la revendication 1, dans lequel lesdits filaments de Nylon sont des monofilaments.

11. Procédé selon la revendication 1, dans lequel ledit premier lot dudit filament de Nylon est immergé dans ladite solution aqueuse pendant moins de 60 min.

12. Procédé selon la revendication 1, dans lequel ledit premier lot dudit filament de Nylon pèse au moins 4,8 kg (10 lbs).
